

COMPOSITIONS,  
COATING OR PLASTIC.

106/86

C. H. SCHOL.

PROCESS OF MAKING LIGHT BRICKS OF BLAST FURNACE SLAG.

APPLICATION FILED DEC. 6, 1911.

1,068,396.

Patented July 22, 1913.



Witnesses:

Charles Thomas  
J. M. Copenhagen.

Inventor:

Carl Heinrich Schol,  
By J. Macmillane

# UNITED STATES PATENT OFFICE.

CARL HEINRICH SCHOL, OF ALLENDORF, GERMANY.

## PROCESS OF MAKING LIGHT BRICKS OF BLAST-FURNACE SLAG.

1,068,396.

Specification of Letters Patent.

Patented July 22, 1913.

Application filed December 5, 1911. Serial No. 664,012.

To all whom it may concern:

Be it known that I, CARL HEINRICH SCHOL, a subject of the German Emperor, and residing at Allendorf, Dillkreis, Germany, have invented a certain new and useful Improved Process of Making Light Bricks of Blast-Furnace Slag, of which the following is a specification.

My invention relates to the manufacture 10 of light bricks and the like of blast-furnace slag.

For manufacturing light bricks and the like, *e. g.* of the type of the well known Rhenish artificial tuff bricks, a filling material of great volume but small density is used which is converted by a suitable binder into a plastic mass from which bricks, slabs and the like can be made and molded by various processes.

20 A primary object of my invention is to provide an improved process of making such light bricks and the like by using blast-furnace slag.

It is well-known to use granulated blast-furnace slag with an admixture of lime for making artificial stone. The process according to my invention differs from the well-known processes in that when using the blast-furnace slag for making light bricks I 30 obtain both the filling material and the binder from blast-furnace slag. When the slag is granulated in the customary manner in part large, very porous and light lumps, and in part granules are formed. According 35 to my invention these bulky but very light lumps are liberated from the granules by sifting. These lumps then form the filling material while the finely ground granules, if necessary mixed with lime, form the 40 binder. The binder is mixed in known manner with the filling material and from this mixture bricks, molded stones, slabs and the like and, indeed, any desired bodies are made in known manner. Owing to the 45 binder setting and hardening the finished brick or the like obtains its strength which by far exceeds that of the tuff bricks on the market at the present day.

According to this process very much 50 greater strength can be obtained when, according to the invention, the lumps of slag serving as filling material are provided with an envelop of cement mortar, whereupon they are left for a long time, if necessary 55 several days, so that the envelop composed of the binding material completely inclos-

ing the lumps has time to harden. The bulky, light and, consequently, relatively weak lumps of slag are incased, as it were, in the slag cement. Owing to this slag 60 cement having time to harden an outwardly very hard, but very light filling material is obtained, which when mixed with the binder forms a mass which is subsequently molded into bricks and the like. The bricks, slabs, 65 and the like thus obtained offer, of course, a very much greater resistance to compression than known bricks of the type described above, so that they can be used for all kinds of building purposes. The same result due 70 to incasing these lumps of slag used as filling material can also be obtained by working up these lumps of slag immediately after the granulating operation. As a rule, blast-furnace slag is led in a liquid state 75 into a reservoir of water where it is quenched and granulated. When fresh, the porous lumps of slag contain approximately 40 to 50% of water. In carrying my invention into practice the binder is added in a dust- 80 like dry state to these wet lumps of slag in the proportion of 1 part binder to 10-12 parts of the porous lumps. The binder and lumps are preferably mixed on a rotary gravity mixer in which the material is 85 mixed for about 4 to 5 minutes. During this time each lump of slag becomes covered with a fine layer of the binder, while its inner pores are still filled with water which subsequently gradually evaporates. These 90 incased lumps of slag are then shot loosely onto a heap.

In order always certainly to obtain as high a percentage as possible of the bulky and loose lumps of slag to be used as filling 95 material when granulating the blast-furnace slag, according to my invention the slag is exposed to the conjoint action of water and air when being granulated. It is well-known to conduct blast-furnace slag directly 100 into water for granulation, and it is also well-known to cause compressed air to act on the stream of slag. In both these cases the formation of the bulky lumps of slag is, however, more or less subject to chance. 105 Now according to my invention water and compressed air are caused to act conjointly on the slag in such manner that an exceedingly high percentage of the filling material is produced.

110 The accompanying drawing diagrammatically shows in sectional elevation one form

of apparatus adapted for carrying my process into practice.

Referring to the drawing, the blast-furnace slag is supplied through the channel *a* 5 into a double-walled tank *b* containing water. The bottom *c* of this tank *b* is perforated like a strainer. Compressed air is supplied through the compressed air pipe *d* into the chamber between the two walls of 10 the tank and passes through the perforations in the bottom *c* so that the slag is exposed to the simultaneous action of water and compressed air. The air must be supplied at such a pressure that the water is prevented 15 from entering into the chamber between the walls of the tank, and the water is constantly kept in a bubbling condition by the fine jets of air entering from below. The lumps of slag and the granules are removed 20 from the tank in well-known manner by the elevator *e*. The scoops of the elevator are preferably perforated in order to allow the lifted water to flow away.

It will be understood that the described 25 apparatus may be substituted by any other suitable device which enables the slag to be exposed to the simultaneous action of compressed air and water.

I claim:—

30 1. The herein-described process of making light bricks of furnace slag, which consists in conducting molten blast-furnace slag into water whereby the molten slag is formed into light bulky lumps and into granules, in 35 separating the lumps from the granules by sifting, in providing the lumps with a hard coat of cement, in mixing the lumps so prepared with a binder, and in forming the mixture thus obtained into bricks.

40 2. The herein-described process of making light bricks of furnace slag, which consists in conducting molten blast-furnace slag into water whereby the molten slag is formed into light bulky lumps and into granules, in 45 separating the lumps while yet wet from the granules by sifting, in mixing the lumps

while yet wet with a dry cement capable of combining with the water in them, in allowing the coating so formed to become hard, in mixing the lumps so prepared with a binder, 50 and in forming the mixture thus obtained into bricks.

3. The herein-described process of making light bricks of furnace slag, which consists in conducting molten blast-furnace slag into 55 water whereby the molten slag is formed into light bulky lumps and into granules, in separating the lumps from the granules by sifting, in providing the lumps with a hard coat of cement, in mixing the lumps so prepared with a binder formed of said granules after being finely ground, and in forming the mixture thus obtained into bricks. 60

4. The herein-described process of making light bricks of furnace slag, which consists 65 in conducting molten blast-furnace slag into water whereby the molten slag is formed into light bulky lumps and into granules, in separating the lumps from the granules by sifting, in providing the lumps with a hard 70 coat of cement, in mixing the lumps so prepared with a binder formed of said granules after being finely ground and an admixture of lime and in forming the mixture thus obtained into bricks. 75

5. The herein-described process of making light bricks of furnace slag, which consists in conducting molten blast-furnace slag into water and simultaneously admitting compressed air into the water whereby the molten slag is formed into light bulky lumps and into granules, in separating the lumps from the granules by sifting, in providing the lumps with a hard coat of cement, in mixing the lumps so prepared, and in forming the mixture thus obtained into bricks. 80

In testimony whereof, I affix my signature in the presence of two witnesses.

CARL HEINRICH SCHOL.

Witnesses:

HENRY HASPER,  
WOLDEMAR HAUPT.

Copies of this patent may be obtained for five cents each, by addressing the "Commissioner of Patents,  
Washington, D. C."